

## UNITED STATES PATENT OFFICE

2,280,082

## MANUFACTURE OF DRYING OILS

Remmet Priester, Deventer, Netherlands, assignor to Naamlooze Venootschap Industrieel Maatschappij Voorheen Noury & Van Der Lande, Deventer, Netherlands, a company of the Netherlands

No Drawing. Application June 13, 1939, Serial No. 278,978. In Great Britain June 20, 1938

15 Claims. (Cl. 106—311)

The invention relates to the manufacture of improved drying oils suitable as media adapted for the production of paints and of impregnating agents. In particular, improved drying oils are obtained by incorporating Isano-oil in drying or semi-drying vegetable or fish oils or products derived from these oils.

Isano-oil, also referred to in the literature under the name "Ongueka-oil," is the oil which occurs in the kernels of the nuts of "Ongueka Klaineane," a tree which belongs to the family of the "Oleaceae," which is very frequently found wild in tropical Africa. Other names for this tree are "Ongueka Gore," "Ongueka des Mponges," "Isano Loango," and "Gore Pahouin."

The raw Isano-oil as such has not the slightest drying properties; these properties only develop after heating.

However, it has now been found that by mixing untreated Isano-oil at room temperature with drying or semi-drying vegetable or fish oils or products derived from these oils, an improved oil may be obtained with quick drying properties and a very good water-resistance. In what direction the improvement is obtained depends on the ratio of the ingredients in the mixture. A rapidly drying oil may be obtained, for example, by mixing linseed oil with Isano-oil in a ratio of 4:1; such a mixture dries in about 48 hours while pure linseed-oil requires, for drying, at least 72 hours.

By increasing the ratio of Isano-oil to linseed oil to about 45 parts of Isano-oil to 55 parts of linseed oil, the drying time is the same as that of pure linseed oil. Such a mixture, however, shows valuable improvements as regards waterproofness and elasticity of the film, which are even better than in the mixture of 1 part of Isano-oil to 4 parts of linseed oil. It seems that with mixtures of Isano-oil and linseed oil a maximum in the speed of drying is obtained by a ratio of 1:4, while a maximum in regard to waterproofness and elasticity is obtained with a ratio of 1:1.

That the acceleration of the speed of drying of linseed oil is indeed due to a particular action of Isano-oil appears clearly from the so-called "Weger" curves. In these curves the increase of weight of the film of the drying oil is plotted against the time during the drying process. Whereas the weight of linseed oil itself increases about 13% during drying, and still increases after the film is dry to about 16-18%, a mixture of Isano-oil and linseed oil (1:4) shows an increase of weight of 9% only. A further particularity is that the dry film of the mixture does not in-

crease in weight but shows a constant weight for a long time, whereas the linseed oil film loses much of its weight in course of time.

A further feature of the cold mixture of a drying oil and Isano-oil in a ratio of 4:1 is the fact that such a mixture has improved wetting properties in respect of pigments; also pigments may be more easily ground with the oil, the paint obtained has a better flow and a high gloss. An ordinary linseed-oil acquires by mixing with Isano-oil the properties of an enamel vehicle.

Also after addition of driers similar results are observed.

## Example 1

15 To a varnish linseed oil, driers are added in a normal quantity such as 0.25% lead, 0.015% cobalt and 0.015% manganese, for instance in the form of naphthenates. Four parts of this oil are mixed with 1 part of Isano-oil and thereafter the drying time of pure linseed oil and the mixture are determined. Whereas the linseed oil is dry after 6½ hours, the mixture dries (under identical conditions) in 4½ hours. The film of the mixture shows a much better waterproofness than that of linseed oil.

## Example 2

1 The same experiment as described in Example 1 was carried out with raw linseed oil, sojabean oil and sardine oil in the mixture. Similar results were obtained as with the experiment in Example 1.

I claim:

35 1. As a new article of manufacture an oil having improved drying properties and comprising Isano-oil and at least one oil selected from the group consisting of drying and semi-drying animal oils and drying and semi-drying vegetable oils.

40 2. An oil having improved drying qualities comprising Isano-oil and at least one oil selected from the group consisting of drying and semi-drying vegetable oils and drying and semi-drying animal oils in a ratio of about 1:4.

45 3. An oil having improved drying qualities comprising Isano-oil and at least one oil selected from the group consisting of drying and semi-drying vegetable oils and drying and semi-drying animal oils, the amount of said Isano-oil being not substantially greater than the amount of said other oil.

50 4. An oil having improved drying qualities comprising Isano-oil and at least one oil selected from the group consisting of drying and semi-

drying vegetable oils and drying and semi-drying animal oils, the amount of said Isano-oil being only a minor fraction of the amount of said other oil.

5. As a new article of manufacture, drying oil which comprises linseed oil and Isano-oil.

6. As a new article of manufacture, drying oil which comprises about four parts of linseed oil and one part of Isano-oil, such oil drying much faster than linseed oil.

7. As a new article of manufacture, drying oil which comprises about 55 parts of linseed oil and about 45 parts of Isano-oil.

8. As a new article of manufacture, drying oil which comprises about equal amounts of linseed oil and Isano-oil, which mixture, after drying, is more water resistant than dried linseed oil.

9. A method of improving the drying qualities of an oil selected from the group consisting of drying and semi-drying animal and vegetable oil which consists in incorporating with the said oils a proportion of Isano-oil.

10. A method of producing an oil having improved drying qualities which consists in mixing

Isano-oil with at least one oil selected from the group consisting of drying and semi-drying vegetable oils and drying and semi-drying animal oils, and a drier.

11. A method of improving the drying qualities of linseed oil which consists in mixing Isano-oil with linseed oil.

12. A method of producing an oil having improved drying qualities which consists in admixing driers with an oil comprising at least one oil selected from the group consisting of the drying and semi-drying animal oils and drying and semi-drying vegetable oils and admixing the said oils with Isano-oil.

13. A drying oil composition which comprises one part of Isano-oil and substantially more than one part of linseed oil.

14. A drying oil composition which comprises one part of Isano-oil and at least one part of linseed oil.

15. A drying oil composition which comprises one part of Isano-oil and at least one part of a fatty oil having drying properties.

REMMET PRIESTER.